

## UNITED STATES PATENT OFFICE

2,150,079

## LUBRICATING COMPOSITION

Carl F. Prutton, Cleveland, Ohio, assignor, by  
means assignments, to The Lubri-Zol Develop-  
ment Corporation, Cleveland, Ohio, a corpora-  
tion of Delaware

No Drawing. Application August 17, 1936,  
Serial No. 96,537

.14 Claims. (Cl. 87—9)

This invention relates, as indicated, to lubricating compositions, and more particularly to compositions for use in connection with the lubrication of the working parts of internal combustion engines, motor vehicles, etc., and it is among the objects of this invention to provide compositions obviating the disadvantages of the usual petroleum oils.

When in use, as in the crank-case of an automobile, for example, it is a well-known fact that oils deteriorate, forming considerable quantities of gummy and semi-solid materials generally included by the term "sludge". This "sludge" thickens the oil, increases friction, lowering the general efficiency of the engine, and necessitates frequent drainage and replacement of the lubricant. In winter the passage of small amounts of gasoline into the crank-case of an engine often results in the precipitation of "sludge" materials which are particularly objectionable since they hinder lubrication of the engine on starting, causing undue wear and starting trouble. Obviously, an oil which does not sludge, under such conditions, would be especially desirable for winter use. The frequent oil changes necessary at all times of the year in order to keep an engine operating efficiently and without danger of injury are a major source of expense and annoyance.

It has been discovered that this "sludge" which forms in the lubricating oil on use contains two predominant components comprising (1) polymerized hydrocarbons and (2) more or less oxidized polymerized hydrocarbons. These components act as cementing agents for small particles of inorganic and insoluble materials, greatly impairing the lubricating effect of the oil. I have found that the best solvents for one component of the "sludge" are not the best for the other. For addition to a lubricating oil it is obvious that solvents must be found which are mutually compatible, soluble or miscible in the oil, and which will dissolve the two components of the "sludge" previously referred to. By lubricating oils are meant mineral oils or their synthetic equivalents.

It is, therefore, among the objects of this invention to provide a lubricant which will not lose its lubricating qualities and suffer other deterioration due to "sludge" formation.

Another object of this invention is to provide a lubricating composition which will not lose its lubricating qualities due to "sludge" formation and will also have extreme pressure characteristics.

It is also among the objects of this invention to provide a lubricating mineral oil which will not deteriorate due to sludge formation and which will be especially effective under conditions of extreme pressure.

Other objects of the invention will appear as the description proceeds.

To the accomplishment of the foregoing and related ends, said invention, then, consists of the means hereinafter fully described and particularly pointed out in the claims.

The following description sets forth in detail certain approved combinations of ingredients embodying my invention, such disclosed means constituting, however, but certain of various forms in which the principle of the invention may be used.

Broadly stated, this invention comprises incorporating at least one each of a halogenated oxygen-free organic compound and an oxygen-bearing organic compound, which is also preferably halogenated, with an oil base.

As is hereinafter more particularly pointed out, the above defined components of the lubricant comprising this invention will preferably and for best results have certain physical and chemical characteristics which especially adapt the same for use in conjunction with the principal types of engines in use today, and for other uses.

The solvent components of the lubricant should be of fairly low volatility, i. e., with a vapor pressure at a temperature of 140° C. of below atmospheric, or preferably a vapor pressure less than atmospheric at a temperature of 170° C. In one embodiment of my invention now in commercial use, one component of my new solvent has a vapor

pressure less than atmospheric at a temperature above 300° C. A mixture of two components, one with a vapor pressure a little below atmospheric at 170° C. and the other with a vapor pressure a little below atmospheric at 350° C., has proven highly satisfactory.

*Oxygen free component*

10 I have found that of the entire class of halogenated oxygen-free organic compounds usable as a component of the solvent constituent in my new lubricant, as above defined, the halogenated hydrocarbons and generally those of the aromatic series are most highly desirable as solvents for the unoxidized polymerized hydrocarbon deposit. Throughout this application the term "aromatic series" is intended to include homologs as well. As hereinafter pointed out, however, certain of the aliphatic compounds of this type are particularly useful for certain purposes.

15 In the case of the halogenated aromatic oxygen-free compounds, it is preferable that the halogen be attached to a carbon atom of the benzenoid ring. These latter compounds are usually more desirable because of their non-corrosive character and general stability.

20 The halogenated oxygen-free organic compounds as noted may be either:

25 A. Aliphatic, such as halogenated:

I. Hydrocarbons.

30 Notably, those containing from four to ten carbon atoms, e. g. fluorinated hexane, fluorinated octane, and fluorinated decane.

II. Amines

35 Primary, secondary and tertiary, e. g. hexylamines, di-amylamines, tri-amylamines, such as: fluorinated tri-amyl amine, fluorinated hexyl amines; also: fluorinated tributyl amine,

40 or the more generally preferable:

B. Cyclic compounds, such as halogenated:

I. Benzene and related compounds such as:

50 (1) Halogenated benzene, e. g. the dichlorbenzenes, notably the ortho compound, the ortho-dibrom benzenes, and the fluorinated benzenes.

55 (2) Halogenated derivatives of benzene such as:

60 (a) Halogenated homologs of benzene, e. g. mono-chlor toluene, mono-chlor xylene, mono chlor cymene, ethyl mono-chlor benzenes, propyl mono-chlor benzenes, di-ethyl dichlor benzenes, propyl dichlor benzenes, and di-ethyl dichlor benzenes.

65 (b) Halogenated amino derivatives of benzene, e. g. chlorinate aniline, mono-chlor aniline (preferably the ortho-compound), mono-chlor di-methyl aniline, chlorinated toluidines, chlorinated xylydines, and chlorinated diphenylamine.

70 (c) Halogenated hydrobenzenes, e. g. hydrogenated dichlor-benzenes, dichlorhexahydrobenzene (dichlor cyclohexane).

II. Polyphenyls, and related compounds, including diphenyl, diphenyl benzenes, etc., such as

(1) Chlorinated diphenyl, e. g. mono-chlor diphenyls, di-chlor diphenyls, and tri-chlor diphenyls.

(2) Brominated diphenyl, e. g. the mono-brom diphenyls.

(3) Fluorinated diphenyl.

(4) Halogenated derivatives of diphenyl, such as:

(a) Halogenated homologs of diphenyl, e. g., chlorinated phenyl-toluenes.

(b) Halogenated amino derivatives of diphenyl, e. g. chlorinated phenyl-anilines, chlorinated phenyl-toluidines, and chlorinated diphenyl amine.

(c) Halogenated hydrodiphenyls, e. g. chlorinated phenyl hexahydrobenzene, and chlorinated dodecahydrodiphenyl.

III. Naphthalene, such as:

(1) Chlorinated naphthalene, e. g.  $\alpha$ -mono-chlor naphthalene.

(2) Brominated naphthalenes, e. g.  $\alpha$ -monobrom naphthalene.

(3) Fluorinated naphthalene.

(4) Halogenated derivatives of naphthalenes, such as:

(a) Halogenated homologs of naphthalenes, e. g. chlorinated methyl naphthalene, notably the alpha compound, chlorinated propyl, and isopropyl substitution products of naphthalene.

(b) Halogenated amine derivatives of naphthalene, e. g. chlorinated naphthylamines, and mono-chlor  $\alpha$ -naphthyl amine.

(c) Halogenated hydronaphthalenes, e. g. chlorinated decahydronaphthalene.

IV. Phenanthrene and anthracene and related compounds, such as:

(1) Chlorinated phenanthrene, chlorinated anthracene.

(2) Halogenated derivatives of phenanthrene and anthracene, such as:

(a) Halogenated homologs, e. g. chlorinated retene, chlorinated 1-methyl phenanthrene, chlorinated 3-methyl phenanthrene, chlorinated 9,10 dimethyl phenanthrene chlorinated propyl and isopropyl derivatives of phenanthrene such as retene, chlorinated dimethyl anthracenes, chlorinated  $\alpha$ -methyl anthracene, chlorinated  $\beta$ -methyl anthracene, and chlorinated propyl and isopropyl derivatives of anthracene.

(b) Halogenated amine derivatives, e. g. chlorinated phenanthryl-amines, and chlorinated anthra-mines.

(c) Halogenated hydrophenanthrenes and halogenated hydroanthracenes, e. g., chlorinated retene oil (contains hydro retene).

5 V. Chrysene, picene, and related compounds, including their derivatives, such as homologs, amine derivatives and other substitution products.

6 VI. Bridged ring compounds, such as the terpenes and related compounds, and their derivatives, e. g. chlorinated pinene.

7 VII. Heterocyclic compounds, such as pyridine, quinoline, pyrrole, thiophene, and derivatives of them, e. g. mono-chlor pyridine.

12 It will be noted that the above enumerated examples of the organic ring compounds which are usually preferred are, in general, compounds of the aryl type, i. e., compounds containing benzenoid ring structures and also of the type in which the halogen is directly attached to an atom which is a part of such ring structure. Very satisfactory results may be obtained when two or more different halogens are present in the same molecule, ortho brom chlor benzene being a good example of such a compound. If the aromatic compounds have been alkylated they are often especially effective.

13 As a matter of convenience, the halogenated diphenyls and substituted diphenyls, as well as halogenated substituted benzenes where two or more phenyl groups are directly linked, may be inclusively referred to as halogenated polyphenyls.

14 Some of the best examples of the aromatic solvents are:

15 Chlorinated benzene, B-I. (1), e. g. di-chlor benzene (notably the ortho compound).  
16 Mono-chlor toluene, B-I. (2) (a).  
17 Chlorinated ethyl benzene.  
18 Chlorinated diphenyl B-II. (1).  
19 Chlorinated aniline B-I. (2) (b).  
20 Chlorinated pyridine B-VIII.  
21 Chlorinated quinoline B-VII.

22 Good examples of halogenated aliphatic hydrocarbons are:

23 Fluorinated pentane.  
24 Fluorinated hexane.  
25 Fluorinated octane.  
26 Halogenated petroleum derivatives, particularly halogenated petroleum waxes.

#### Oxygen-bearing component

27 I have found that of the entire class of oxygen-bearing organic compounds usable as a component in my improved solvent as above defined the halogenated compounds and preferably those of the aromatic series are generally superior solvents for the oxidized polymerized hydrocarbon deposit, and that these solvents may be used in conjunction with the solvents for the unoxidized polymerized hydrocarbon deposit, also being compatible with the oil. Here again compounds of the aromatic series with the halogen attached to the ring are favored. However, a certain number of the oxygen-bearing aliphatic compounds have been found to be very effective.

28 The oxygen-bearing components may, for convenience, be classified as follows:

#### 70 I. Aliphatic, or carbon chain type.

##### Oxygen-bearing derivatives of:

- A. Hydrocarbons of the paraffin series;
- B. Hydrocarbons of the olefine series; and
- 75 C. Hydrocarbons of the acetylene series.

#### II. Organic ring type.

##### Oxygen-bearing derivatives of:

- A. "Carbon ring" type compounds.
  - (a) Of the aromatic, or allied type, including oxygen-bearing derivatives of benzene, naphthalene, anthracene, etc., also compounds of the bridged ring type, such as the terpenes, and related compounds.
  - (b) Of the class including the cyclo-paraffins, cyclo-olefines, etc. Examples of this class are oxygen-bearing derivatives of the following:

(1) Hydrogenation products of benzene (e.g. cyclohexane, cyclohexene, cyclohexadiene), such as hydrogenated phenol notably cyclohexanol, di-hydro phenol, tetra-hydro phenol.

(2) Hydrogenation products of naphthalene (e. g., decahydronaphthalene, tetrahydronaphthalene, etc.), such as the hydrogenated naphthols.

(3) Naphthalenes, such as naphthalenic acid, etc.

(c) Of mixed type such as derivatives of indene, hydrindene, hydranthracene, etc.

#### B. "Heterogeneous ring" type compounds.

(a) Of the aromatic or allied type including derivatives of pyridine, quinoline, etc.

(b) Other types such as furan and its derivatives and derivatives of thiophene, pyrrole, etc.

The oxygen-bearing derivatives of the foregoing compounds may also be classified according to the nature of the attachment of the oxygen to the molecule, viz.:—

#### I'. Directly attached to one or more carbon atoms, as in the case of:

- (1') Ethers and analogous compounds.
- (2') Compounds containing the



50

radicle, such as alcohols and other derivatives of carbinol (including phenols, cresols, naphthols, etc.).

(3') Compounds containing the carbonyl



55

radicle, such as aldehydes, ketones, organic acids, esters and salts of organic acids, thio-acids and esters of thio-acids.

(4') Compounds in which oxygen forms a part of the ring structure, e. g., furan and its derivatives, anthraquinone, etc.

II'. Indirectly attached through the means of some other atom, i. e., in the form of an inorganic radicle, e. g.: amide, arsenate, arsenite, chlorate, chloride, cyanate, hydroxylamine, hypochlorite, nitrate, nitrite, nitro, nitroso, oxime, perchlorate, phosphate, phosphite, sulphate, sulphite, sulphonic acid, sulphide, sulphoxide, thio-phosphate, and thio-sulphate.

70

60

65

75

The following table indicates some of the compounds which are especially suitable, halogenated or unhalogenated, as the case may be:

Organic oxygen compounds

|       | Ring compounds                                       | Unhalogenated                                                                                                                                                                                                                                                                                                                                                                               | Halogenated                                                                                                                                                                     |
|-------|------------------------------------------------------|---------------------------------------------------------------------------------------------------------------------------------------------------------------------------------------------------------------------------------------------------------------------------------------------------------------------------------------------------------------------------------------------|---------------------------------------------------------------------------------------------------------------------------------------------------------------------------------|
| 5     | Aromatic phenols                                     | Phenol<br>α-naphthol<br>Amino phenols<br>Butyl phenol<br>Phenyl phenol<br>Xylenol<br>"Tar acids" (preferably refined by distillation)                                                                                                                                                                                                                                                       | o-Chlor phenol<br>Monochlor α-naphthol                                                                                                                                          |
| 10    | Alcohols                                             | Benzyl alcohol                                                                                                                                                                                                                                                                                                                                                                              | Chlor benzyl alcohol                                                                                                                                                            |
| 15    | Aldehydes (less desirable because of polymerization) | Phenyl ethyl alcohol<br>Benzaldehyde                                                                                                                                                                                                                                                                                                                                                        |                                                                                                                                                                                 |
| 20    | Ketones                                              | Benzophenone<br>Phenyl tolyl ketones<br>Diphenyl ketone<br>Acetanilide<br>Stearanilide<br>Phenyl fatty acids, e. g. phenyl acetic acid                                                                                                                                                                                                                                                      | Mono-chlor benzophenone                                                                                                                                                         |
| 25    | Amides                                               |                                                                                                                                                                                                                                                                                                                                                                                             | Chlorphenyl acetic acid                                                                                                                                                         |
| Acids |                                                      |                                                                                                                                                                                                                                                                                                                                                                                             | Chlor-salicylic acid<br>Ethyl chlorbenzoates<br>Butyl chlorbenzoates<br>Diethyl chlorphthalates<br>Dibutyl chlorphthalates<br>Ethyl and butyl esters of chlorphenyl acetic acid |
| 30    | Esters                                               | Methyl salicylate<br>Benzyl acetate<br>Pyridine acetate<br>Quinoline acetate<br>Diphenyl ether                                                                                                                                                                                                                                                                                              | Methyl chlor salicylates<br>Chlorbenzyl acetates                                                                                                                                |
| 35    | Ethers                                               | Phenyl ethyl ether<br>Dixenyl ether<br>Dinaphthyl ether<br>Alkylated diphenyl ether                                                                                                                                                                                                                                                                                                         | Chlorinated diphenyl ether<br>Chlorphenyl ethyl ethers<br>Chlorinated dixenyl ether<br>Chlorinated dinaphthyl ether<br>Alkylated chlor diphenyl ether                           |
| 40    | Non-aromatic oxygen bearing organic ring compounds   | Cyclo-hexanol<br>Naphthenic acids<br>Esters of naphthenic acids<br>Oxygen-bearing heterocyclic compounds<br>(1) Furane and derivatives, e. g. esters of pyromuic acid (furoates), furfuryl alcohol and esters of it, e. g. furfuryl acetate,<br>(2) Oxygen bearing derivatives of thiophene and pyrrole, e. g. esters of thiophene carboxylic acids and esters of pyrrole carboxylic acids. |                                                                                                                                                                                 |
| 45    | Chain compounds                                      | Octyl alcohol<br>Decyl alcohol<br>Lauryl alcohol<br>Cetyl alcohol<br>Methyl stearate<br>Lauryl acetate<br>Tri-ethanol-amine acetate<br>Tri-lauryl phosphate<br>Tri-ethanol amine<br>Tri-butanol amine<br>Butyl ether<br>Amyl ether<br>Octyl ether<br>Dipropyl ketone<br>Dibutyl ketone<br>Di-amyl ketone<br>Di-octyl ketone<br>Propionic acid<br>Butyric acid<br>Lauric acid                | Fluorinated octyl alcohol<br>Fluorinated decyl alcohol<br>Fluorinated lauryl alcohol<br>Fluorinated cetyl alcohol<br>Methyl dichlor stearate                                    |
| 50    |                                                      |                                                                                                                                                                                                                                                                                                                                                                                             |                                                                                                                                                                                 |
| 55    |                                                      |                                                                                                                                                                                                                                                                                                                                                                                             |                                                                                                                                                                                 |
| 60    |                                                      |                                                                                                                                                                                                                                                                                                                                                                                             |                                                                                                                                                                                 |
| 65    |                                                      |                                                                                                                                                                                                                                                                                                                                                                                             |                                                                                                                                                                                 |
| 70    |                                                      |                                                                                                                                                                                                                                                                                                                                                                                             |                                                                                                                                                                                 |
| 75    |                                                      |                                                                                                                                                                                                                                                                                                                                                                                             |                                                                                                                                                                                 |

A good example of a solvent of the oxygen-bearing class is chlorinated diphenyl ether, containing an average of from about three to about eight atoms of halogen per molecule. Chlorinated diphenyl ether which contains about six atoms of chlorine per molecule, and has preferably been purified by vacuum distillation, or other means, is one of the most desirable solvents of this class. This solvent boils at a temperature above 300° C. without appreciable decomposition. (See my co-pending application Ser. No. 83,976.)

Of the above enumerated classes of oxygen-bearing compounds, the aromatic compounds are generally preferred and particularly the aromatic ethers and ketones. Another preferred class of compounds is that in which oxygen forms a part of a ring structure. In the case of unhalogenated oxygen-bearing organic compounds they should boil at atmospheric pressure without appreciable decomposition.

Since aromatic compounds containing multiple ring structures of the condensed type such as naphthalene, anthracene, penanthranene, etc. (that is, of the type in which certain carbon atoms are contained in or common to two rings) are more easily oxidized, and, therefore, less stable than the "non-condensed" multiple-ring type in which no carbon atoms are thus shared, the latter type is to be preferred. Poly-nuclear aromatic compounds (that is, those containing more than one ring) of the non-condensed type are thus the more desirable of such aromatic compounds.

It is to be noted that certain compounds of the class in which oxygen is in the form of an inorganic radicle, have the additional advantage of inhibiting corrosion, and therefore otherwise corrosive halogenated oxygen-free organic compounds may be used in conjunction with them for service in lubricants. Notable examples of such compounds are the organic phosphates, of which tri-cresyl phosphate is a good example, and the phosphites, such as tri-phenyl phosphite. However, with these exceptions the oxygen is generally preferred on the form of an organic radicle.

Preferred combinations to make up my new solvent include: about 25% to 75% o-dichlor benzene with one or more of the following:

|                           |    |
|---------------------------|----|
| Hexachlor diphenyl oxide  | 55 |
| Trichlor diphenyl oxide   |    |
| Monochlor benzophenone    |    |
| Benzophenone              |    |
| Phenyl acetate            |    |
| Phenol                    |    |
| o-Phenyl phenol           |    |
| Cyclo hexanol             |    |
| Dibutyl phthalate         | 60 |
| Methyl salicylate         |    |
| Lauryl alcohol            |    |
| Methyl stearate           |    |
| Tri-ethanol amine         |    |
| Tri-ethanol amine acetate | 65 |

The chlorinated diphenyl oxide compounds referred to above are compounds containing an average number of chlorine atoms equivalent to that indicated.

Chlorine, bromine, and fluorine are the halogens most desirable in both the oxygen-free and oxygen-containing compounds, fluorine forming particularly stable compounds which are no longer so difficult to prepare as formerly. Methods of preparing fluorine compounds which will be found

satisfactory for use in my solvent are described, for instance, in U. S. Patent No. 2,013,030, Example IV, and in U. S. Patent No. 2,013,050, Example X. My invention, of course, is not to be considered as involving any particular method of preparation of the components nor is it intended to be limited by any such method or methods. Chlorine is the least expensive and most commercially available of all the halogens, and bromine is also satisfactory, although considerably more expensive, as is iodine.

As the exact manner in which my solvent constituents act upon the "sludge" is not entirely understood, I do not intend my invention to be restricted by any explanation or theory. However, it seems that the two types of solvents mutually aid one another in attacking the gummy "sludge" for it has been found that the effectiveness of their joint action is more than the cumulative effect of the two when used separately. The presence of the halogen lowers the volatility and thus enables the use of a number of the most effective solvents which would otherwise be too highly volatile at engine temperatures. The presence of the halogen also notably enhances the solvent action of the compounds and therefore makes available more effective compounds. The degree of halogenation may, however, reach an optimum beyond which further halogenation gives no improvement in the solvent action or may even cause a decline in effectiveness.

The solvent action of my new lubricant may sometimes be improved by the use of a more or less complex mixture of one or both of the two solvent addition components used. This complexity may result from (a) the production of a plurality of compounds obtained by the halogenation process, as, for example, the chlorination of diphenyl which is capable of producing a large number of chlorine bearing compounds differing as to the number and location of the chlorine atoms in the molecule; or (b) the use of a product resulting from the halogenation of a complex organic material such as certain still fractions and solvent-extraction fractions obtained in the separation of petroleum products and coal-tar products.

It is also of advantage to use a combination of solvent components which will have a fairly wide range of volatility. This assures a certain and uniform solvent action, even if some of the components should be partially volatilized by unexpectedly high temperatures.

The relative proportions of halogenated oxygen-free organic constituents and oxygen-bearing organic constituents in the new solvent comprising my invention may vary within wide limits, depending upon the particular materials used, a very minor proportion of the more active components at times being quite effective, the kind of oil to which the solvent is to be added, and the kind of engine employing the lubricant. The ratio of the amount of halogenated oxygen-free organic constituents to the amount of oxygen-bearing organic material usually may vary from about one to ten, up to about ten to one, but preferably only from about one to two, up to two to one. For most applications a lubricating composition containing a solvent comprising substantially equal amounts of each type has been found very satisfactory.

The amount of the solvent combination to be added to the oil will depend upon the type of oil and the type of engine using the lubricant, and may vary over wide limits, for example, from

about .001% to about 20% by weight based on the oil. To obtain a maximum of desirable characteristics in the lubricant, a proportion of from about .1% to about 3% of the combined solvent is usually of advantage while amounts up to 5 or 10% are occasionally desirable and amounts up to 20% may often be used without unduly decreasing the viscosity of the lubricant.

Proper stability of the components of the solvent combination in the lubricant is an important factor. Since the materials are to be exposed to relatively high temperatures in the crank-case, etc., they should be particularly resistant to thermal decomposition.

Resistance to hydrolysis is a most desirable characteristic because of the likelihood of a certain amount of moisture being present in the crank-case. Under these conditions, easily hydrolyzed halogen compounds will tend to produce hydrogen halides which will cause corrosion of the parts of the engine with which they come in contact.

The superiority of my lubricant has been demonstrated commercially by its highly successful use in automobile, truck and bus engines. The solvent constituents may be most conveniently introduced into the mineral oil before such oil is placed in the crank-case, but this invention does not cover nor is it intended to be limited by any particular method of addition of the solvent constituents to the lubricant. Any practicable means of addition is intended to be within the scope of this invention. Other specific applications of this invention have been made and will occur to those acquainted with the art and this invention is intended to include all such applications.

To a mineral oil base are therefore added my solvent constituents comprising at least one representative of each of the two types of compounds disclosed to inhibit the formation and aid in removal of oil "sludge". It is distinctly preferable, but not absolutely necessary, that at least one of the solvents be of the aromatic series. The two solvent compositions described have a co-operative dissolving effect, each enabling the other to work more quickly and completely.

This invention is equally applicable to other than automotive fields of lubrication and other uses for my improved lubricant will be immediately apparent to those skilled in the art. This invention is intended to cover all such applications.

It is also to be noted that combinations of the type described are highly effective in increasing the extreme pressure characteristics of the lubricant, and thus my improved lubricant has the combined advantages of being non-sludging, even in cold weather, and at the same time providing the safety of an extreme pressure lubricant.

This application is a continuation in part of my copending applications Ser. Nos. 737,070, filed July 26, 1934, and 755,987, filed December 4, 1934.

Other modes of applying the principle of my invention may be employed instead of the one explained, change being made as regards the materials employed in carrying out the process, provided the ingredient or ingredients stated in any of the following claims or the equivalent of such stated ingredient or ingredients be employed.

I therefore particularly point out and distinctly claim as my invention:

1. A lubricating composition containing as a principal lubricating constituent a major amount

of mineral lubricating oil with the properties of such composition affecting its use as a lubricant improved by incorporating therein a total amount of at least .1%, based on the amount of mineral oil, of both an oil-soluble halogenated oxygen-free aromatic compound and an oil-soluble organic oxygen compound, the proportion of each of said compounds being less than 20% based on the amount of said mineral lubricating oil and 10 said compounds being of the type which will not substantially evaporate from such lubricating composition at ordinary temperatures.

15 2. A lubricating composition containing as a principal lubricating constituent a major amount of mineral lubricating oil with the properties of such composition affecting its use as a lubricant improved by incorporating therein a total amount of at least .1%, based on the amount of mineral oil, of both an oil-soluble chlorinated aromatic hydrocarbon and an oil-soluble saponifiable organic oxygen compound, the proportion of each of said compounds being less than 20% based on the amount of said mineral lubricating oil and said compounds being of the type which will not substantially evaporate from such lubricating composition at ordinary temperatures.

3. A lubricating composition containing as a principal lubricating constituent a major amount of mineral lubricating oil with the properties of such composition affecting its use as a lubricant improved by incorporating therein a total amount of at least .1%, based on the amount of mineral oil, of both an oil-soluble halogenated oxygen-free organic ring compound and an oil-soluble saponifiable organic oxygen compound, the proportion of each of said compounds being less than 20% based on the amount of said mineral lubricating oil and said compounds being of the type which will not substantially evaporate from such lubricating composition at ordinary temperatures.

40 lubricating composition at ordinary temperatures.

4. A lubricating composition containing as a principal lubricating constituent a major amount of mineral lubricating oil with the properties of such composition affecting its use as a lubricant improved by incorporating therein a total amount of at least .1%, based on the amount of mineral oil, of both an oil-soluble halogenated oxygen-free aromatic compound and a stable oil-soluble 45 saturated organic oxygen compound, the proportion of each of said compounds being less than 20% based on the amount of said mineral lubricating oil and said compounds being of the type which will not substantially evaporate from such lubricating composition at ordinary temperatures.

50

55 atures.

56 5. A lubricating composition containing as a  
57 principal lubricating constituent a major amount  
58 of mineral lubricating oil with the properties of  
59 such composition affecting its use as a lubricant  
60 improved by incorporating therein a total amount  
61 of at least .1%, based on the amount of mineral  
62 oil, of both an oil-soluble chlorine bearing oxy-  
63 gen-free substituted benzene and an oil-soluble  
64 organic oxygen compound, the proportion of  
65 each of said compounds being less than 20%  
66 based on the amount of said mineral lubricat-  
67 ing oil and said compounds being of the type  
68 which will not substantially evaporate from such  
69 lubricating composition at ordinary temperatures.

70 6. A lubricating composition containing as a principal lubricating constituent a major amount of mineral lubricating oil with the properties of such composition affecting its use as a lubricant improved by incorporating therein a total amount 75 of at least .1%, based on the amount of mineral

oil, of both a chlorinated benzene and an oil-soluble organic oxygen compound, the proportion of each of said compounds being less than 20% based on the amount of said mineral lubricating oil and said compounds being of the type which will not substantially evaporate from such lubricating composition at ordinary temperatures.

7. A lubricating composition containing as a principal lubricating constituent a major amount of mineral lubricating oil with the properties of such composition affecting its use as a lubricant improved by incorporating therein a total amount of at least .1%, based on the amount of mineral oil, of both ortho-dichlorbenzene and an oil-soluble organic oxygen compound, the proportion of each of said compounds being less than 20% based on the amount of said mineral lubricating oil and said compounds being of the type which will not substantially evaporate from such lubricating composition at ordinary temperatures. 20

8. A lubricating composition containing as a principal lubricating constituent a major amount of mineral lubricating oil with the properties of such composition affecting its use as a lubricant improved by incorporating therein a total amount of at least .1%, based on the amount of mineral oil, of both an oil-soluble halogenated oxygen-free organic ring compound and halogenated diphenyl oxide, the proportion of each of said compounds being less than 20% based on the amount of said mineral lubricating oil and said compounds being of the type which will not substantially evaporate from such lubricating composition at ordinary temperatures. 20 26 30

9. A lubricating composition containing as a principal lubricating constituent a major amount of mineral lubricating oil with the properties of such composition affecting its use as a lubricant improved by incorporating therein a total amount of at least .1%, based on the amount of mineral oil, of both ortho-dichlorbenzene and chlorinated diphenyl oxide, the total proportion of said compounds being within their combined solubility in said mineral lubricating oil.

10. A lubricating composition containing as a principal lubricating constituent a major amount of mineral lubricating oil with the properties of such composition affecting its use as a lubricant in the crank case of an internal combustion engine improved by incorporating therein a total amount of at least 1%, based on the amount of mineral oil, of both a stable oil-soluble halogenated oxygen-free aromatic compound and a stable oil-soluble organic oxygen compound, the proportion of each of said compounds being less than 20% based on the amount of said mineral lubricating oil and said compounds having a vapor pressure below atmospheric at a temperature of 140° C.

140 C. 11. A lubricating composition containing as a principal lubricating constituent a major amount of mineral lubricating oil with the properties of such composition affecting its use as a lubricant in the crank case of an internal combustion engine improved by incorporating therein a total amount of at least .1%, based on the amount of mineral oil, of both a stable oil-soluble halogenated organic compound and a stable oil-soluble oxygen-free aromatic oxygen compound, the proportion of each of said compounds being less than 20% based on the amount of said mineral lubricating oil and said compounds having a vapor pressure below atmospheric at a temperature of 170° C.

12. A lubricating composition containing as a 75

principal lubricating constituent a major amount of mineral lubricating oil, the sludge solventicity of which is improved by incorporating therein an effective minor amount of both an oil-soluble 5 halogenated oxygen-free aromatic compound and an oil-soluble organic oxygen compound, the proportion of each of said compounds being within their combined solubility in said mineral lubricating oil and said compounds being of the 10 type which will not substantially evaporate from such lubricating composition at ordinary temperatures.

13. A lubricating composition containing as a principal lubricating constituent a major amount 15 of mineral lubricating oil with the properties of such composition affecting its use as a lubricant improved by incorporating therein a total amount of at least .1%, based on the amount of mineral oil, of both an oil-soluble halogen bearing oxygen-free aromatic compound and an oil-soluble 20 organic oxygen compound, the total proportion of

each of said compounds being less than 5%, based on the amount of mineral oil, the ratio of the amounts of said compounds being from about 1 to 10, up to about 10 to 1, and said compounds being of the type which will not substantially 5 evaporate from such lubricating composition at ordinary temperatures.

14. A lubricating composition containing as a principal lubricating constituent a major amount of mineral lubricating oil with the properties of such composition affecting its use as a lubricant improved by incorporating therein a total amount of at least .1%, based on the amount of mineral oil, of both an oil soluble halogen bearing oxygen-free aromatic compound and an oil-soluble ester, 10 the total proportion of each of said compounds being less than 20%, based on the amount of mineral oil and said compounds being of the type 15 which will not substantially evaporate from such lubricating composition at ordinary temperatures. 20

CARL F. PRUTTON.

CERTIFICATE OF CORRECTION.

Patent No. 2,150,079.

March 7, 1939.

CARL F. PRUTTON.

It is hereby certified that error appears in the printed specification of the above numbered patent requiring correction as follows: Page 3, first column, line 41, for "B-VIII" read B-VII; page 6, first column, line 35, claim 3, strike out the word "saponifiable"; and second column, line 68, claim 11, for "organic" read oxygen-free aromatic; line 69, same claim, for "oxygen-free aromatic" read organic; page 7, first column, lines 7 and 8, claim 12, for "within their combined solubility in" read less than 20% based on the amount of; and that the said Letters Patent should be read with this correction therein that the same may conform to the record of the case in the Patent Office.

Signed and sealed this 18th day of April, A. D. 1939.

Henry Van Arsdale.

Acting Commissioner of Patents.

(Seal)

principal lubricating constituent a major amount of mineral lubricating oil, the sludge solventicity of which is improved by incorporating therein an effective minor amount of both an oil-soluble 5 halogenated oxygen-free aromatic compound and an oil-soluble organic oxygen compound, the proportion of each of said compounds being within their combined solubility in said mineral lubricating oil and said compounds being of the 10 type which will not substantially evaporate from such lubricating composition at ordinary temperatures.

13. A lubricating composition containing as a principal lubricating constituent a major amount 15 of mineral lubricating oil with the properties of such composition affecting its use as a lubricant improved by incorporating therein a total amount of at least .1%, based on the amount of mineral oil, of both an oil-soluble halogen bearing oxygen-free aromatic compound and an oil-soluble 20 organic oxygen compound, the total proportion of

each of said compounds being less than 5%. based on the amount of mineral oil, the ratio of the amounts of said compounds being from about 1 to 10, up to about 10 to 1, and said compounds being of the type which will not substantially 5 evaporate from such lubricating composition at ordinary temperatures.

14. A lubricating composition containing as a principal lubricating constituent a major amount of mineral lubricating oil with the properties of 10 such composition affecting its use as a lubricant improved by incorporating therein a total amount of at least .1%, based on the amount of mineral oil, of both an oil soluble halogen bearing oxygen-free aromatic compound and an oil-soluble ester, 15 the total proportion of each of said compounds being less than 20%, based on the amount of mineral oil and said compounds being of the type which will not substantially evaporate from such lubricating composition at ordinary temperatures. 20

CARL F. PRUTTON.

CERTIFICATE OF CORRECTION.

Patent No. 2,150,079.

March 7, 1939.

CARL F. PRUTTON.

It is hereby certified that error appears in the printed specification of the above numbered patent requiring correction as follows: Page 3, first column, line 41, for "B-VIII" read B-VII; page 6, first column, line 35, claim 3, strike out the word "saponifiable"; and second column, line 68, claim 11, for "organic" read oxygen-free aromatic; line 69, same claim, for "oxygen-free aromatic" read organic; page 7, first column, lines 7 and 8, claim 12, for "within their combined solubility in" read less than 20% based on the amount of; and that the said Letters Patent should be read with this correction therein that the same may conform to the record of the case in the Patent Office.

Signed and sealed this 18th day of April, A. D. 1939.

Henry Van Arsdale.

Acting Commissioner of Patents.

(Seal)